

3,684,426

LEVELLING POLYAMIDE FIBER DYEING WITH SULFONATED LONG CHAIN ALKYL DIPHENYL ETHER AND QUATERNIZED LONG CHAIN ALKYL AMMONIUM ALKYLENE OXIDE CONDENSATE

Jakob Bindler, 63 Kilchgrundstrasse, and Rudolf Keller, 32 Kilchgrundstrasse, both of Riehen, Switzerland  
No Drawing. Filed Mar. 2, 1970, Ser. No. 15,841  
Int. Cl. D06p 3/06

U.S. Cl. 8—15

8 Claims

ABSTRACT OF THE DISCLOSURE

A process for the even, non-streaky dyeing of fibre material made from synthetic polyamide of differing dyestuff-affinity, such as textured polyamide fibre material, is disclosed, which comprises pre-treating said fibre material, at a pH-value of from 2 to 7 and at temperatures of from 30 to 130° C., with aqueous solution of a mixture of auxiliaries consisting of at least one mono- or di-sulphonated higher-alkyl-diphenylether as anion-active compound and at least one cation-active, non-quaternated or quaternated compound containing at least one basic nitrogen atom to which are bound at least one polyglycol ether chain and at least one aliphatic radical having from 10 to 18 carbon atoms, the molecule containing from 8 to 20 di-alkylene-oxy groupings, and, optionally, further auxiliaries normally used in dyeing, adding then, at temperatures of from 30 to 100° C., pre-dissolved anionic dyestuff, and completing the dyeing in the heat. By this process, even on polyamide fibre material tending to exhibit streakiness upon dyeing, even and non-streaky dyeings are obtained with, in themselves, poorly levelling dyestuffs, with extensive exhaustion of the dye bath.

DETAILED DISCLOSURE

The present invention relates to a process for the even, non-streaky dyeing of fibre material made from synthetic polyamide of differing dyestuff-affinity, as well as to the fibre material dyed using this process.

It has been found that fibre material made from synthetic polyamide having differing dyestuff-affinity, such as textured polyamide fibre material, e.g. Banlon, can be dyed very evenly and non-streakily by pre-treating this fibre material, at a pH-value of from 2 to 7 and at temperatures of from 30 to 130° C., preferably at 40 to 95° C., with the aqueous solution of a mixture of auxiliaries, consisting of

(a) at least one anion-active compound of Formula I,



wherein

R represents an alkyl radical having from 8 to 18 carbon atoms,

X represents a cation and

n represents a number from 1 to 2,

(b) at least one cation-active, non-quaternated or quaternated compound containing at least one basic nitrogen atom, to which are bound at least one polyglycol ether chain and at least one aliphatic radical having from 10 to 18 carbon atoms, whereby the molecule contains from 8 to 20 groupings of Formula II,



as well as, optionally,

(c) further auxiliaries normally used in dyeing, adding then, at temperatures of from 30 to 100° C., pre-dissolved anionic dyestuff and completing the dyeing in the heat, preferably at boiling temperature or at temperatures above 100° C., under pressure.

Anion-active compounds of Formula I are known per se and can be produced, e.g. by the methods described in British Pats. Nos. 912,340 and 1,043,043, by reacting correspondingly substituted diphenyl ethers together with a sulphonating agent, such as sulphur trioxide or chlorosulphonic acid, in the solution of a poly-chlorinated aliphatic hydrocarbon, or by dissolving the diphenyl ether compound in a saturated aliphatic hydrocarbon and then bringing it into contact with the sulphonating agent.

Anion-active compounds of Formula I which have proved particularly valuable, in the process according to the invention, are those wherein R represents an alkyl radical having from 9 to 12 carbon atoms, X represents an alkali metal ion, such as the lithium or potassium ion, preferably, however, the sodium ion, or the ammonium ion and n represents the number 2. Disulphonated compounds of Formula I, which are obtained by sulphonating the 4-dodecylphenyl ether, are especially preferred.

The cation-active, non-quaternated or quaternated compounds (b), usable in the process according to the invention, are likewise known per se and can be produced in a manner known per se, e.g. by reaction of the corresponding aliphatic amines, especially long-chain primary alkyl-mono-, -di- or -tri-amines, the alkyl or alkenyl radical of which contains from 10 to 18 carbon atoms, such as dodecyl-, octadecyl- or octadecenylamine, dodecylpropyl-enediamine, octadecylethylenediamine and octadecylidihydroxyethylenetriamine, with alkylene oxides, e.g. with propylene oxide, but particularly with ethylene oxide, and, optionally, subsequent reaction with usual quaternating agents such as methyl-, ethyl- or benzylhalides, diethyl sulphate and, in particular, dimethyl sulphate. Suitable cation-active compounds (b), usable according to the invention, are also products obtained by reaction of the above mentioned alkylamines with from 1 to 2 equivalents of styrene oxide, from 0 to 2 equivalents of propylene oxide and from 1 to 19 equivalents of ethylene oxide as well as, optionally, subsequent quaternisation.

Cation-active compounds of Formula III are preferred,



wherein

R<sub>1</sub> represents an alkyl or alkenyl radical having from 10 to 18 carbon atoms, especially the octadecenyl or the octadecyl radical,

R<sub>2</sub> represents a lower alkyl radical having from 1 to 4 carbon atoms, particularly the methyl group,

of Y<sub>1</sub> and Y<sub>2</sub>, one Y represents hydrogen and the other Y represents hydrogen or the phenyl radical,

m represents 0 or 1,

n and p represent whole numbers, the sum of which is from 6 to 20, especially from 11 to 18, and

A represents an anion, particularly the methosulphate ion.

The sum of the coefficients n and p represents a mean value, and there are present mixtures of analogous compounds with polyalkyleneoxy substituents of varying chain-length.

Anionic dyestuffs, suitable for the process according to the invention, can belong to very diverse classes of dyestuffs. These can be, for example, the commercially im-

portant dyestuff classes of the azo, anthraquinone, phthalocyanine, nitro or formazane dyestuffs which can also contain metals bound in complex linkage such as copper, nickel, chromium or cobalt. Suitable azo dyestuffs are, principally, monoazo dyestuffs, e.g. of the type phenylazobenzene, phenylazonaphthalene, phenylazohydroxy- or -aminopyrazole, phenylazoacylacetylarylamide, or those of the analogous naphthylazo series, whereby the aromatic nuclei can be suitably substituted. Also suitable are dis- and polyazo dyestuffs. The azo dyestuffs, to which also belong the formazane dyestuffs, can be metallised, principally by chromium or cobalt, but also by copper or nickel, whereby 1 or 2 dyestuff molecules per metal ion participate in the complex.

The pH-value of the dye bath is adjusted to the desired value by the addition of an acid, such as acetic acid, formic acid or sulphuric acid. The preliminary treatment of the fibre material in the dye bath containing the auxiliaries as defined, preferably lasts 5 to 30 minutes. The weight ratio of anion-active to cation-active compound is thereby advantageously from 1:1 to 10:1.

After the preliminary treatment, the acidity of the dye liquor can be reduced by the addition of an acid-binding agent, such as an alkali metal hydroxide, -carbonate or -hydrogen carbonate, by the addition of ammonium hydroxide, disodium or dipotassium phosphate, sodium or potassium acetate, as well as by the addition of hexamethylenetetramine.

An advantageous embodiment of the process, according to the invention, consists in carrying out the preliminary treatment at boiling temperature, then adding the predissolved dyestuff and completing the dyeing at the same temperature. After the dyeing is completed, the dyed material is advantageously rinsed in the usual manner, if necessary given an aftertreatment to improve the fastness to wet processing, and dried.

In general, the anion-active compounds are used in amounts of from 0.1 to 5% by weight, relative to the fibre material to be treated, preferably in amounts of from 0.2 to 2% by weight. The cation-active compounds are, in general, used in amounts of from 0.01 to 2% by weight, preferably in amounts of from 0.05 to 0.5% by weight.

As auxiliaries which are normally used in dyeing, the dye bath can contain, e.g. urea, thiourea, thiadiethyleneglycol or hydrophilic compounds having limited water-solubility such as, e.g. butyl alcohol or benzyl alcohol.

Further additives are textile-protective agents having affinity to the fibres and which protect the textile material to be dyed.

Suitable fibre materials made from synthetic polyamide, which can be dyed using the process according to the invention, are, e.g. condensation products from hexamethylenediamine and adipic acid (Polyamide 6.6) or sebacic acid (Polyamide 6.10) or mixed condensation products, e.g. from hexamethylenediamine, adipic acid and  $\epsilon$ -caprolactam (Polyamide 6.6/6), also the polymerisation products from  $\epsilon$ -caprolactam, known under the trade names of Polyamide 6, "Perlon," "Grilon" or "Enekalon," or from  $\omega$ -aminoundecanoic acid (Polyamide 11 or "Rilsan"). These fibres can be used at any stage of processing, that is to say, e.g. in the form of threads, yarns, knitted goods and fabrics.

The process, according to the invention, is distinguished in that, even on polyamide fibre material tending to exhibit streakiness upon dyeing, even and non-streaky dyeings are obtained with, in themselves, poorly levelling dyestuffs, with extensive exhaustion of the dye bath.

The temperatures are given in degrees centigrade in the following examples.

#### EXAMPLE 1

To 200 ml. of softened water are added 0.1 ml. of 40% acetic acid and 0.1 g. of a mixture, consisting of 0.076 g. of a 45% aqueous solution of the disodium salt

of the dodecyldiphenyl ether disulphonic acid, 0.0075 g. of a compound of the formula



of the dodecyldiphenyl ether disulphonic acid, 0.015 g. of a compound of the formula



and 0.033 g. of water.

To the obtained auxiliary liquor are added 10 g. of knitted fabric made from textured polyamide-6.6 yarn, the temperature of the liquor is rapidly raised, with continuous movement of the textile material, up to the boiling point and boiling is maintained for 30 minutes. To the liquor are then added 0.050 g. of the dyestuff of the formula,



0.018 g. of the dyestuff of the formula



(Synthesized in U.S. Pat. 2,714,103.)

and 0.014 g. of the dyestuff of the formula



(Synthesized in Belgium Pat. 674,050.)

pre-dissolved in 20 g. of water. Boiling proceeds for a further 60 minutes until the dyestuff has drawn onto the textile material. The material is afterwards rinsed warm and then cold, and dried. The resulting brown dyeing is smooth and level and differences in affinity, caused by the material, are extremely well equalised.

Without the addition of the above mixture of auxiliaries, applying otherwise the same procedure, an uneven and very streaky dyeing is obtained.

If, in the above example, the 0.015 g. of the compound of the formula



are replaced by the same amount of one of the cation-active compounds listed in the second column of the following Table II, the procedure being otherwise as de-

scribed in the above example, then similarly level and non-streaky dyeings are obtained on knitted fabric made from textured polyamide-6.6 yarn.

TABLE II

| Ex. No. | Cation-active compound                                                                                                                                                                     |
|---------|--------------------------------------------------------------------------------------------------------------------------------------------------------------------------------------------|
| 10..... | $(CH_2CH_2O)_nH$<br>$C_{12}H_{25}-N$<br>$\quad\quad\quad (CH_2CH_2O)_pH$<br>$n+p=10$                                                                                                       |
| 15..... | $(CH_2CH_2O)_nH$<br>$C_{12}H_{25}-N$<br>$\quad\quad\quad (CH_2CH_2O)_pH$<br>$CH_3SO_4^-$<br>$n+p=8$                                                                                        |
| 20..... | $(CH_2CH_2O)_nH$<br>$C_{16}H_{37}-N$<br>$\quad\quad\quad (CH_2CH_2O)_pH$<br>$Br^-$<br>$n+p=20$                                                                                             |
| 25..... | $(CH_2CH_2O)_nH$<br>$C_{16}H_{37}-N$<br>$\quad\quad\quad (CH_2CH_2O)_pH$<br>$C_4H_9$<br>$n+p=20$                                                                                           |
| 30..... | $(CH_2CH_2O)_nH$<br>$C_{18}H_{35}-N-CH_2CH_2CH_2-N$<br>$\quad\quad\quad (CH_2CH_2O)_sH$<br>$\quad\quad\quad (CH_2CH_2O)_tH$<br>$n+p+z=20$                                                  |
| 35..... | $(CH_2CH_2O)_nH$<br>$C_{18}H_{35}-N-CH_2CH_2-N-CH_2CH_2-N$<br>$\quad\quad\quad (CH_2CH_2O)_sH$<br>$\quad\quad\quad (CH_2CH_2O)_tH$<br>$\quad\quad\quad (CH_2CH_2O)_uH$<br>$n+p+z_1+z_2=20$ |
| 40..... | $(CH_2CH_2O)_nH$<br>$C_{18}H_{35}-N$<br>$\quad\quad\quad (CH_2CH_2O)_pH$<br>$SO_4CH_3^-$<br>$n+p=10$                                                                                       |
| 45..... | $(CH_2CH_2O)_nH$<br>$C_{18}H_{35}-N$<br>$\quad\quad\quad (CH_2CH_2O)_pH$<br>$Cl^-$<br>$n+p=10$                                                                                             |
| 50..... | $(CH_2CH_2O)_nH$<br>$C_{18}H_{35}-N$<br>$\quad\quad\quad (CH_2CH_2O)_pH$<br>$Cl^-$<br>$n+p=10$                                                                                             |

## EXAMPLE 13

Muffs made from polyamide-6 textured yarn are introduced into an open dyeing apparatus (packing machine). An about 40° warm auxiliary liquor is prepared separately which contains, relative to the weight of the textile material, 2.0% of 40% acetic acid and 3.0% of the mixture of auxiliaries used in Example 1 (ratio of goods to liquor ca. 1:15).

This auxiliary liquor is pumped into the dyeing apparatus. The temperature of the auxiliary liquor is then rapidly raised to 96° and the material to be dyed is treated at this temperature for 30 minutes. The pH-value of the dye bath is thereupon raised to 6.0 by the addition of aqueous ammonia solution. After the auxiliary liquor has been thoroughly mixed, an addition is made, relative to

the weight of textile material, of 0.5% of the dyestuff of the formula



which is pre-dissolved in ten times the amount of water, and dyeing proceeds for a further 60 minutes at 96°. The red dyed material is then rinsed warm and afterwards cold, and dried.

A knitted fabric, produced from the thus dyed yarn, is free of streaks and is uniform.

#### EXAMPLE 14

To 300 ml. of water at 70° are added 0.5 g. of the mixture of auxiliaries, used in Example 5, and 0.2 ml. of 85% formic acid. 10 g. of tricot made from polyamide-6.6 textured yarn are pre-treated at 70° for 15 minutes in the obtained auxiliary liquor. To the auxiliary liquor are then added 0.04 g. of the dyestuff of the formula



(Synthesized in Canadian Pat. 579,201 and Belgian Pat. 554,509).

dissolved in 4 ml. of water, and the dye liquor is heated to boiling within 20 minutes. Whilst continuous movement of the material being dyed is maintained, dyeing proceeds during one hour at the boiling temperature, after which the obtained brown dyeing is rinsed and dried.

The resulting dyeing is appreciably more level than a dyeing obtained without addition of the above-mentioned mixture of auxiliaries.

What we claim is:

1. A process for the even, non-streaky dyeing of fibre material made from synthetic polyamide of differing dye-stuff-affinity, which comprises

(I) applying to said fibre material, at a pH-value of from 2 to 7 and at temperatures of from 30 to 130° C., with the aqueous solution of a mixture of auxiliaries comprising

(a) at least one anion-active compound of Formula I



wherein  
R represents an alkyl radical having from 8 to 18 carbon atoms,  
X represents a cation, and  
n represents a number from 1 to 2, and

(b) at least one cation-active compound of the formula



wherein

R1 represents an alkyl or alkenyl radical having from 10 to 18 carbon atoms,

R2 represents a lower alkyl radical having from 1 to 4 carbon atoms,

of Y1 and Y2, one Y represents hydrogen and the other Y represents hydrogen or the phenyl radical,

m represents 0 or 1

n and p represents whole numbers, the sum of which is from 6 to 20, and

A represents an anion; and

(II) adding, at temperatures of from 30 to 100° C., pre-dissolved anionic dyestuff and completing the dyeing at the temperature of 30 to 100° C.

35. 2. A process as claimed in claim 1 wherein the aqueous solution contains further dyeing auxiliaries.

3. A process as claimed in claim 1 wherein in the anion-active compounds R represents an alkyl radical having from 9 to 12 carbon atoms, X represents an alkali metal ion or the ammonium ion, and n represents the number 2.

4. A process as claimed in claim 1 employing a weight ratio of anion-active to cation-active compounds of from 1:1 to 10:1.

45. 5. A process as claimed in claim 1 wherein the preliminary treatment is carried out at a temperature of between 40 and 95° C.

6. A process as claimed in claim 1 wherein the dyeing is performed at boiling temperature.

7. A process as claimed in claim 1 wherein the dyeing is performed at temperatures above 100° C. under pressure.

8. A process as claimed in claim 1 wherein the preliminary treatment is carried out at boiling temperature, the pre-dissolved dyestuff then added and the dyeing then completed at the same temperature.

#### References Cited

##### UNITED STATES PATENTS

|           |         |        |        |
|-----------|---------|--------|--------|
| 2,623,806 | 12/1952 | Fuchs  | 8-21 B |
| 2,967,755 | 1/1961  | Keller | 8-84   |
| 3,086,832 | 4/1963  | Casty  | 8-84   |

##### OTHER REFERENCES

Brooks: Defensive Publication of application S.N. 661,820, 895 O.G. 41.

Schmidlin: Preparation and Dyeing of Synthetic Fibers, pp. 172-173, pub. by Chapman & Hall Ltd., London, 1963.

DONALD LEVY, Primary Examiner

U.S. Cl. X.R.

UNITED STATES PATENT OFFICE  
CERTIFICATE OF CORRECTION

Patent No. 3,684,426 Dated August 15, 1972

Inventor(s) Jakob Bindler and Rudolph Keller

It is certified that error appears in the above-identified patent and that said Letters Patent are hereby corrected as shown below:

Column 1, line 2 under the title, after "Switzerland",  
please insert:  
-- assignors to Ciba-Geigy AG, Basel, Switzerland --;

column 1, between lines 3 and 4, under the title, please  
insert: -- claims priority, application Switzerland,  
March 24, 1969, Serial No. 4381 --.

Column 5, please change the first formula from the bottom  
to read as follows: --  $C_{18}H_{35}$  -- instead of  $C_{18}H_{37}$  as  
printed.

Column 6, Table II, Example No. 10, please change  
" $n+p+Z_1+Z_2=20$ " to --  $n+p+Z_1+Z_2=18$  --;

column 6, third line from the bottom, please change "dye"  
to -- auxiliary --.

Signed and sealed this 19th day of February 1974.

(SEAL)

Attest:

EDWARD M. FLETCHER, JR.  
Attesting Officer

C. MARSHALL DANN  
Commissioner of Patents